

## UNITED STATES PATENT OFFICE

2,526,771

## COUNTERLIVERING AGENT IN RED LEAD PAINT

Richard B. Pollak, Maywood, Calif.

No Drawing. Re-filed for abandoned application  
Serial No. 607,480, July 27, 1945. This application  
February 13, 1948, Serial No. 8,283

4 Claims. (Cl. 106—258)

1

My invention relates to preparations containing red lead and although applicable also to preparations wherein the red-lead-carrying vehicles are alkyd resins, phenolic resins, poly-amine resins or natural resins, alone or in any combination, the invention is especially applicable to red-lead-in-oil paints and pastes and inks, the oil vehicle being often linseed oil. It is applicable also to preparations wherein the red lead is only one of a plurality of pigments.

This application is re-filed for my inadvertently abandoned application, Serial No. 607,480, filed July 27, 1945, and is identical therewith, with respect to the descriptive parts of the two applications.

The invention concerns itself with the problem of livering, which is defined as the progressive increase in the viscosity of a red-lead paint or the like on ageing, to a degree appreciably in excess of the original viscosity, namely, that at the time of manufacture. The period free of livering may be as long as one year or as brief as a few days, depending on the marketing and use conditions. This thickening reaches a point where the material has solidified so much as to be no longer usable.

The livering is undesirable, not only because of the labor necessary for thinning the more or less solidified substance, but also because, under certain conditions, an excessive thinning is required and, as a result whereof, a thinner paint film with less hiding power and with less resistance against corrosion and abrasion results, and one therefore of shorter life.

The expedient of packing red lead pigment separately from the vehicle for mixing by the user immediately before application, constitutes more of an escape from rather than a solution of the problem. The reason is that it is time-consuming for the user and, additionally, results are not consistent in that this expedient imposes too great a responsibility on the average user, with reference to his care and skill in selecting the correct proportions, not to mention the possibility of using a poor or unsuitable kind of oil, and not to mention frequently preparing too much.

It is known to the industry, in the case of red lead preparations, that livering is caused primarily by the presence of litharge (lead monoxide) and which, even in small quantities, is a deleterious impurity in association with red lead, whose formula is  $Pb_3O_4$ .

In the manufacture of red-lead-in-oil according to Federal Specification TT-P-86, amend-

2

ment 1 of September 1, 1943, livering is frequently encountered if the acid number of the linseed replacement oil (Federal Specification TT-O-371) is 4.0 or above. In fact, if the roller mill gets hot or if the paste is not immediately reduced, livering can occur with replacement oil of acid number 3.0. Paint manufacturers who formerly produced red lead of 85% purity, the impurity being mainly litharge, have in the 10 course of years been forced to gradually increase the red lead content for the paint trade to 95 and 97%. As a result of this improvement, the livering tendency has been appreciably lowered, but the fact remains that, even with the 97% 15 grade, manufacturers find themselves inconveniently restricted in their choice of suitable vehicles. Also, even when a generally suitable vehicle is employed, it will not infrequently react unfavorably in the presence of only slightly abnormal conditions.

To partly counteract the reactive tendency, it was also general practice to cook the vehicle under a near vacuum or under an inert gas like nitrogen or carbon dioxide, or under normal atmospheric pressure but with low temperature over a longer period. However, every one of the foregoing methods adds considerably to the cost and reduces the output from any given equipment.

Briefly described, my invention consists of adding, to a production batch of red-lead-in-oil or red lead in any other vehicle, a counter-livering agent of the class of glycol ethers. The glycol ethers can be used, as I discovered previously to 35 conceiving the instant invention, to restore already livered paints by adding to them 0.25% or over of any one or more, in combination, of the glycol ethers, said proportions being on the basis of weight as are all other references thereto herein. Satisfactory results were obtained also, by the addition of 1% or more of an alcohol, such as ethyl, isopropyl, secondary butyl, or normal butyl alcohol. Accompanying the thinning action by the alcohol, was the eventual bad settling out on the part of the pigment, which result did not occur with the glycol ethers.

In the course of experiments for restoring livered paints, I discovered that a glycol ether can be added to the batch when manufacturing it, and, if in suitable proportion, the glycol ether keeps the paint or paste or ink or the like sufficiently fluid for a desired period between manufacture and use. If the proportion of glycol ether 50 is too small, the product will still progressively

body with age, and if too high, bad settling will result.

In the case of one particular 85% red lead-in-oil paste, which in the absence of the counter-livering agent, livered solid two hours after manufacture, the incorporation of 0.25% of a glycol ether prevented livering. The paste so treated, was found to be still fluid at the end of one week. The amount of glycol ether that should be added, in any given case, is determined by a number of factors, among them, the amount of litharge, the reactivity of the vehicle, the manufacturing process employed in making the red lead, and the length of the pre-livering period that is desired.

In no case, have I found that less than 0.25% of glycol ether is effective. With most preparations, I have found a percentage of about 1% suitable. With increases over 1%, the tendency of the red lead pigment to settle becomes increasingly pronounced until, when glycol ether is used in a quantity greater than 4%, the settling rate becomes excessive, even in the case of low litharge content. To sum up, I have found a range of from 0.25% to 4% of glycol ether, relatively to the amount of red lead, more or less satisfactory, conditioned, by the lengths of the periods between manufacture and use.

In the class of glycol ethers, any one of them or any number of them may be used in any combination and in any proportions relatively to one another to constitute a total glycol ether content within the limits stated as a counter-livering agent. Among the various glycol ethers, which are occasionally referred to also as ether-alcohols, I have used with equal success, singly and in various combinations, as counter-livering agents, appropriately respectively to different pre-livering periods, "Cellosolve" (mono-ethyl ether of ethylene glycol), "Methyl Cellosolve" (mono-methyl ether of ethylene glycol), "Butyl Cellosolve" (mono-butyl ether of ethylene glycol), and "Carbitol" (mono-ethyl ether of diethylene glycol).

This discovery now makes possible the manufacturing of ready-mixed red-lead paints from dry red lead of higher litharge content, hitherto unsuitable for such manufacture. Furthermore, it will now be possible to manufacture ready-mixed red-lead paints with higher acid oils and

varnishes, eliminating the necessity to body the oils or cook the varnishes under atmospheres of inert gases, or to body them under low temperatures requiring much longer cooking schedules. Furthermore, the method may be used with many other types of paints, whereby many materials whose use hitherto has been impractical because of livering tendencies, may now be used.

To eliminate the need to otherwise employ alternative terms, the expression, a fluidly applicable covering medium containing red lead, can be appropriately employed to describe red lead paints, pastes, inks, and the like, and whether in an oil or other vehicle.

15 There is claimed:

1. An organic surface coating consisting essentially of a pigment consisting of the oxide or hydroxide of lead, a vehicle containing a drying glyceride oil which, in the absence of a counter-livering agent, will cause livering, and at least one lower saturated aliphatic ether-alcohol, the weight of total ether-alcohol being not less than 0.25% and not more than 4% of said pigment.

25 2. A non-livering pigmented composition consisting essentially of a pigment consisting of the oxide or hydroxide of lead, a vehicle containing a drying glyceride oil which, in the absence of a counter-livering agent, will cause livering, and at least one lower saturated aliphatic ether-alcohol, the weight of total ether-alcohols being not less than 0.25% and not more than 4% of the weight of said pigment.

30 3. A non-livering pigmented composition consisting essentially of a pigment consisting of the oxide or hydroxide of lead, a vehicle containing a drying glyceride oil which, in the absence of a counter-livering agent, will cause livering, and the mono-butyl ether of ethylene glycol, the weight of total glycol-ether being not less than 0.25% and not more than 4% of said pigment.

40 4. An organic surface coating consisting essentially of a pigment consisting of the oxide or hydroxide of lead, a vehicle containing a drying glyceride oil which, in the absence of a counter-livering agent, will cause livering, and the mono-butyl ether of ethylene glycol, the weight of total glycol ether being not less than 0.25% and not more than 4% of said pigment.

RICHARD B. POLLAK.

No references cited.